

## 1

3,065,526

**MATERIAL FOR HANDLING MOLTEN GLASS**  
 James S. Hill, Cranford, N.J., assignor, by mesne assignments, to Engelhard Industries, Inc., Newark, N.J., a corporation of Delaware  
 No Drawing. Original application Oct. 25, 1957, Ser. No. 692,257, now Patent No. 2,973,283, dated Feb. 28, 1961. Divided and this application Sept. 10, 1958, Ser. No. 760,061

2 Claims. (Cl. 29—199)

The present invention deals with an apparatus for handling molten glass as, for example, glass forming dies or extrusion nozzles for the spinning of glass fibers.

Alloys of platinum with up to about 50 percent rhodium have been suggested and used for the manufacture of many types of spinning nozzles for artificial fibers, these alloys combining the required properties for the purpose, to a large extent, such as hardness and corrosion resistance.

However, for apparatus handling molten glass, such as e.g. glass spinnerettes, a further requirement for satisfactory operation becomes important, i.e., the surface which is in contact with the molten glass should not be wetted thereby. This requirement is not satisfactorily met by the platinum-rhodium alloys used heretofore. On the other hand, it is known that platinum-gold alloys show a considerable resistance to wetting by molten glass, but they are mechanically insufficiently resistant, especially at the high temperature of molten glass.

It has been found that the desired properties of hardness, and of non-wetting by molten glass, can be obtained by depositing, for example by electroplating or any other suitable method, a double coating upon an article of a platinum-rhodium alloy, which may be the portion of an apparatus which contacts molten glass, such as a spinnerette for spinning glass fibers, a die in a press or the like.

According to the invention, the article is coated with platinum, and then a coating of gold is applied upon the platinum layer whereupon the article is heated to diffusion temperature, preferably by placing it in a furnace at about 800° C. and gradually raising the temperature to about 1200° C. The heat treatment causes the metals to diffuse into each other whereby, in the different boundary zones, solid solutions are formed, thus insuring that the coatings adhere firmly to each other and to the platinum-rhodium surface.

The coatings of platinum and gold may be in the range of about 0.0001 to about 0.001 inch and good results have been obtained with layers of about 0.0005 inch.

Moreover, it has been found by tests made with platinum-rhodium alloys containing 10 percent to 40 percent by weight rhodium that the surfaces obtained display a combination of properties which the single components do

## 2

not show. The surfaces are extremely repellent to molten glass, due to the predominating content of gold in the outer layer, wherein some platinum but practically no rhodium is present, but at the same time the hardness is increased beyond the hardness the original platinum-rhodium alloy would have attained, when subjected to the same heat treatment, without being coated or if coated with one of the components only.

It is believed that this result is due to the formation of solid solutions which are gradually enriched in gold near the surface whereas an increasing content of rhodium is present deeper in the metal. The intermediate layer of platinum prevents undesirable diffusion between the rhodium content of the alloy and the gold coating, thus acting simultaneously as a buffer and as a bonding agent between the platinum-rhodium alloy and the gold layer.

It will be obvious to those skilled in the art that many modifications may be made within the scope of the present invention without departing from the spirit thereof, and the invention includes all such modifications.

This application is a division of co-pending application Serial No. 692,257 filed October 25, 1957, now Patent No. 2,973,283.

What is claimed is:

1. A material for handling molten glass and resistant to wetting by molten glass, composed of an alloy of platinum and from 10 percent to 50 percent rhodium with a coating on a surface thereof composed of interdiffused layers of platinum and gold with the platinum on the platinum-rhodium surface and the gold on the platinum and each of the layers having a thickness of up to 0.001", and the surface of the coating having a hardness at least equal to the platinum-rhodium alloy.
2. A material according to claim 1, wherein the platinum and gold layers are electroplated layers.

## References Cited in the file of this patent

## UNITED STATES PATENTS

|           |            |       |               |
|-----------|------------|-------|---------------|
| 111,551   | Kearsing   | ----- | Feb. 7, 1871  |
| 145,274   | Blake      | ----- | Dec. 9, 1873  |
| 1,460,888 | Cook       | ----- | July 3, 1923  |
| 1,659,757 | Aderer     | ----- | Feb. 21, 1928 |
| 1,704,126 | Fry        | ----- | Mar. 5, 1929  |
| 1,947,180 | Bart       | ----- | Feb. 13, 1934 |
| 1,963,910 | McIntyre   | ----- | June 19, 1934 |
| 2,106,527 | Hostetter  | ----- | Jan. 25, 1938 |
| 2,190,296 | Richardson | ----- | Feb. 13, 1940 |
| 2,391,457 | Carlson    | ----- | Dec. 25, 1945 |
| 2,460,547 | Stevens    | ----- | Feb. 1, 1949  |
| 2,803,925 | Klausmann  | ----- | Aug. 27, 1957 |
| 2,949,633 | Drummon    | ----- | Aug. 23, 1960 |